

# UNITED STATES PATENT OFFICE.

ELTON R. DARLING, OF MONTCLAIR, NEW JERSEY, ASSIGNOR, BY DIRECT AND MESNE ASSIGNMENTS, TO ESSEX LABORATORIES, INC., A CORPORATION OF NEW YORK.

## PROCESS OF MAKING TITANIUM OXID.

1,315,011.

Specification of Letters Patent.

Patented Sept. 2, 1919.

No Drawing.

Application filed January 18, 1919. Serial No. 271,915.

To all whom it may concern:

Be it known that I, ELTON R. DARLING, a citizen of the United States, residing at Montclair, in the county of Essex and State of New Jersey, have invented certain new and useful Improvements in Processes of Making Titanium Oxid, of which the following is a specification.

This invention relates to a process of making titanium oxid from rutile or other titaniferous ores, preferably from those with a comparatively high titanium oxid content.

In carrying out my process I may proceed in the following illustrative manner:  
15 A quantity of finely powdered rutile, preferably of about 120 mesh is exposed to a heat of about 125° centigrade or above, preferably 150° centigrade, in the presence of chlorin gas, thus forming the chlorid of titanium in a volatilized condition, which is then passed into a boiling solution of glucose, whereby the oxid of titanium is formed, leaving as a by-product a solution of glutaric acid which is valuable for certain commercial purposes. The oxid of titanium is then filtered, washed and dried.

The process may be performed in a continuous manner by keeping the glucose in the solution in slight excess, and continuing 30 the operation until a nearly saturated solution of the glutaric acid is obtained.

Ilmenite or other titaniferous ore may be used in place of rutile, but I prefer to use the latter on account of its much higher 35 titanium oxid content. I may use a solution of fructose or other mono-saccharoses in place of glucose although I prefer glucose on account of its lesser cost.

While it is preferable to use a finely powdered ore, it is possible to carry on the operation with ores in a coarser form.

The solution of glucose or other mono-saccharose may be under the boiling point, although the operation is expedited by using 45 it at the boiling point or over.

What I claim is:—

1. The process of making titanium oxid which consists of exposing finely powdered titaniferous ore to a high heat in the presence of chlorin gas, and passing the volatilized titanium chlorid into a solution of glucose, thus forming titanium oxid, and then filtering, washing and drying this product so as to form a fine dry powder.

55 2. The process of making titanium oxid

which comprises exposing powdered titaniferous ore to a high heat in the presence of chlorin gas, thus forming volatilized titanium chlorid, which is then passed into a solution of a mono-saccharose, thus forming titanium oxid and then filtering, washing and drying this product so as to form a fine, dry powder.

3. The process of making titanium oxid which consists of exposing powdered titaniferous ore to a temperature of 125° C. or more in the presence of chlorin gas, thus forming volatilized titanium chlorid, which is then passed into a solution of glucose, whereby titanium oxid is formed, and then 60 filtering, washing and drying this product so as to form a fine, dry powder.

4. The process of making titanium oxid which comprises heating powdered titaniferous ore to a temperature of 125° C. or over in the presence of chlorin gas, thus forming volatilized titanium chlorid, which is then passed into a solution of one of the mono-saccharoses whereby titanium oxid is formed; and then filtering, washing and 70 drying the product so as to form a fine, dry powder.

5. The process of making titanium oxid in a continuous manner which comprises heating powdered titaniferous ore to a temperature of 125° C. or over, in the presence of chlorin gas, thus forming the chlorid of titanium in a volatilized condition, and then passing the volatilized chlorid of titanium into a boiling solution of glucose, whereby 85 the oxid of titanium is formed, and in keeping the glucose in the solution in slight excess, and continuing the operation until a nearly saturated solution of glutaric acid is obtained.

6. The process of making titanium oxid and glutaric acid which comprises heating powdered titaniferous ore to a temperature of 125° C. or over, in the presence of chlorin gas, thus forming the chlorid of titanium 100 in a volatilized condition, and then passing the volatilized chlorid of titanium into a boiling solution of glucose, whereby the oxid of titanium and glutaric acid are formed, and in separating these products.

7. In the process of making titanium oxid, the steps which consist in heating a powdered titaniferous ore to a high temperature in the presence of chlorin gas, thus forming volatilized titanium chlorid, and 110

then passing the volatilized titanium chlorid into a solution of a mono-saccharose, whereby titanium oxid is formed.

8. In the process of making titanium oxid, 5 the steps which consist in heating a powdered titaniferous ore to a high temperature in the presence of chlorin gas, thus forming volatilized titanium chlorid, and then passing the volatilized titanium chlorid into a 10 boiling solution of a mono-saccharose, whereby titanium oxid is formed.

9. The process of making titanium oxid which consists in heating a finely divided titaniferous ore to a temperature of 125° C. 15 or over in the presence of chlorin gas, thus forming volatilized titanium chlorid; and then passing the volatilized titanium chlo-

rid into a boiling solution of a mono-saccharose, whereby titanium oxid is formed; and then filtering, washing and drying the 20 product so as to form a fine, dry powder.

10. The process of making titanium oxid and glutaric acid which comprises heating powdered titaniferous ore to a temperature of 125° C. or over, in the presence of chlorin 25 gas, thus forming the chlorid of titanium in a volatilized condition, and then passing the volatilized titanium chlorid into a boiling solution of a mono-saccharose whereby the oxid of titanium and glutaric acid are 30 formed, and in separating these products and filtering, washing and drying the oxid of titanium so as to form a fine, dry powder.

ELTON R. DARLING.